

Jan. 17, 1939.

E. GERLACH

2,144,370

METHOD OF CUTTING BODIES SOLUBLE IN LIQUID

Filed July 3, 1937



INVENTOR  
ERWIN GERLACH

BY *H. Shrover*  
ATTORNEY

## UNITED STATES PATENT OFFICE

2,144,370

## METHOD OF CUTTING BODIES SOLUBLE IN LIQUID

Erwin Gerlach, Berlin, Germany, assignor to Telefunken Gesellschaft für Drahtlose Telegraphie m. b. H., Berlin, Germany, a corporation of Germany

Application July 3, 1937, Serial No. 151,951  
In Germany July 10, 1936

5 Claims. (Cl. 125—21)

This invention relates to a method of cutting thin layers from bodies which are soluble in liquid, in particular crystals such as Rochelle salt or other crystals.

5 Bodies soluble in liquid are usually cut by means of a thread moistened with the solvent of the body to be cut. When cutting bodies in accordance with this method it was found that the cut surface is often unclean. It is especially at 10 at the edges of the body to be cut and past which the thread moves that the liquid carried with the thread is rubbed off. But this liquid left behind at the body eats into the surface of the crystal and it is especially the edges that are particularly exposed to this action. In piezo-electric 15 crystals such as produced, for instance, of Rochelle salt, it is an absolute requirement that the edges of the crystal are clean and exact.

According to the invention a clean, unobjectionable cut surface and a possible rapid cutting through the body to be cut through can be assured if the following conditions have the proper relationship.

The material of the thread depends on the 25 body to be cut through. In case of Rochelle salt, a thread of artificial silk was found to be an especially favorable material, yet also threads of rubber are well suited for the cutting. Of further importance is the speed of the thread. The latter depends on the material of the thread 30 and on the thickness of the body to be cut. Then the amount of solvent applied to the thread is also of significance. At the place of cutting, the thread should be not too moist and not too wet. Also, at this place, the amount of liquid to be applied depends on the type of the body to be cut 35 and on its thickness. Finally, the feed is to be set according to the type and thickness of the body to be cut.

40 The optimum cutting must be ascertained by tests for the respective kind of material to be cut.

For Rochelle salt and a cutting length of about 12 mm. and with a thread of artificial silk having a thickness of about 0.5 mm., favorable results have been obtained at a cutting speed (feed) ranging from 1 to 4 mm./min., a supply of liquid ranging from 2 to 16 mm./sec. and a velocity of the thread from 1 to 3 m./sec.

45 The figure shows schematically an example of a cutting arrangement for carrying out the method according to the invention.

The endless thread 5 is placed around four rollers 1, 2, 3 and 4. The roller 1 is driven by a motor not shown in the figure. There is disposed

between the rollers 1 and 4 the supply nozzle 6 for the liquid solvent of the body to be cut, for instance, a crystal of Rochelle salt. The supply of the solvent can be controlled, but this control arrangement is not shown herein. Between the 5 rollers 3 and 4 the crystal 7 is clamped into a support moved upon the thread 5 in the direction of the arrow.

The operation during cutting is as follows:

The solvent flows out of the nozzle 6 upon the 10 thread 5, the latter moving in the direction indicated by the arrow. When the thread moves over the driver roller 1 a part of the liquid is being thrown off, and this partial throwing off of the liquid from the thread occurs also when the 15 latter passes over the other rollers. After leaving the roller 3, the thread passes over the crystal slightly loosening up the same at the place of cutting. Care must be taken that the thread is maintained in a partly moist and partly dry 20 state, that is, it must not carry too large an amount of liquid solvent, otherwise, a non-saturated solution will be deposited at the place at which the thread leaves the crystal. As a result thereof, the crystal is subjected to eating by 25 said solution especially at the edges of the cut surface of the crystal.

When the thread leaves the crystal, the liquid still present on the thread is practically saturated with crystal molecules. Then the thread 30 passes again over the roller 4 finally to be moved again past the nozzle 6 through which it is being moistened again whereby the solution thereon will be diluted.

The quantity of solvent dripped onto the 35 thread will, as previously pointed out, be partly thrown off when the thread 5 moves over the drive roller 1. The amount of liquid remaining on the thread is capable of dissolving further quantities of the body material to be cut, since 40 the said liquid is in the non-saturated state.

If necessary in place of the four rollers shown in the example, also a smaller number of rollers or more than four rollers may be used. Thus, a larger number of guide rollers may be necessary, 45 where a larger amount of liquid is to be applied to the thread at the place of the nozzle in order that a possibly large number of dissolved molecules will be thrown off by the thread. In this way, the liquid on the thread can dissolve at the 50 place of cutting a sufficient number of molecules of the body to be cut.

In place of the endless thread passing in the same direction, a thread which carries out a reciprocating movement may be used. In this

case, two nozzles are preferably to be employed, the crystal being disposed between the two nozzles. Also, in this case it is necessary that saturated solution be removed from the thread.

5. What is claimed is:

1. Method of cutting Rochelle salt crystals by means of a thread moistened with a solvent of the body to be cut, characterized in that by using an endless thread of artificial silk with a thickness of about 0.5 mm. for cutting the crystal, the cutting speed (feed) is 1 to 4 mm/min., the liquid supply 2 to 16 mm<sup>2</sup>/sec. and the speed of the thread 1 to 3 m/sec. at a cutting length of about 12 mm.

15. 2. Apparatus for cutting Rochelle salt crystals comprising a first roller, a second roller, a third roller and a fourth roller, an endless thread placed around said rollers, means for driving at least one of said rollers, means for keeping

20. said endless thread moistened by a liquid solvent of said crystal, said last mentioned means located between said first and fourth rollers, and a support for the crystal to be cut located between said third and fourth rollers.

25. 3. Apparatus for cutting Rochelle salt crystals comprising a first roller, a second roller, a third roller and a fourth roller, an artificial endless thread placed around said rollers, means for

driving at least one of said rollers, means including a nozzle for keeping said endless thread moistened by a liquid solvent of said crystal, said last mentioned means located between said first and fourth rollers, and a support for the crystal to be cut located between said third and fourth rollers.

4. Apparatus for cutting Rochelle salt crystals comprising a first roller, a second roller, a third roller and a fourth roller, an endless thread 10 placed around said rollers, means for driving at least one of said rollers, means for keeping said endless thread moistened by a liquid solvent of said crystal, said last mentioned means located between said first and fourth rollers, and a clamp 15 for supporting said crystal to be cut and located between said third and fourth rollers, said clamp having means for moving the crystal toward said thread.

5. Apparatus for cutting piezo-electric crystals 20 comprising a plurality of rollers, an endless thread placed around said rollers, means for driving at least one of said rollers, means for keeping said endless thread moistened by a solvent of said crystal, and means for supporting said crystal in a position to be cut by said endless thread.

ERWIN GERLACH.